

1

2,928,712

**MOLTEN UREA DYEING PROCESS**

Samuel Nelson Bradshaw, Coventry, England, assignor to Courtaulds Limited, London, England, a British company

No Drawing. Application June 26, 1957  
Serial No. 668,043

Claims priority, application Great Britain May 26, 1953

8 Claims. (Cl. 8—85)

This invention relates to the dyeing of textile materials. This application is a continuation-in-part application of my application Serial No. 428,375, filed May 7, 1954, now abandoned.

In the normal dyeing procedure, textile materials are treated with an aqueous solution or dispersion of a dyestuff which is substantive to the material at a temperature depending on the nature of the material being dyed and the materials are left in the dyebath for a considerable period and are then rinsed and dried. The dyebath may also contain one or more dyeing assistants, for example common salt or Glauber's salt or other compounds which assist the material in taking up the dye and give a uniform penetration of the material by the dye. In the normal dyeing process therefore water is the usual medium in which the dye is transferred to the textile materials.

The object of the present invention is to improve the dyeing of organic textile materials.

According to the present invention a process for dyeing organic textile materials comprises impregnating the textile material with a solution of urea and with an aqueous solution or dispersion of at least one dyestuff which is soluble in molten urea and is substantive to the textile material, drying the textile material at a temperature below the melting point of urea (132° C.), heating the dried material in the absence of steam at a temperature between the melting point of urea and 160° C. to melt the urea whereby it serves as a solvent for the dyestuff, from which resultant solution transfer of the dyestuff to the material takes place, washing the dyed material to remove the urea and again drying the material.

An essential feature of this invention is that molten urea is used instead of water as the dyestuff transfer medium.

In a preferred method of carrying out the invention the textile materials are impregnated with a single solution of urea in which the dyestuff is either dissolved or dispersed, the impregnated material is dried at a temperature below the melting point of urea and then baked at a temperature above the melting point of the urea, this baking being essentially a dry heating in the absence of steam. The impregnation is preferably effected at room temperature. The textile materials may, however, be first impregnated with a solution of urea and then with a solution or dispersion of a dyestuff. The bath or baths are preferably aqueous although other solvents than water, e.g. alcohol or aqueous alcohol, may be used. The preferred take-up of urea by the textile material is 40–55 percent by weight based on the weight of the dry textile material. The drying of the impregnated material is preferably effected at about 80° C. After the baking

2

the dyed textile materials are washed to remove the urea and then dried.

The process of the present invention is suitable for dyeing with dyestuffs which are soluble in molten urea for example direct cotton dyestuffs, dispersed acetate dyestuffs, soluble acetate dyestuffs, leuco esters of vat dyestuffs, aggregated acid dyestuffs and metal complex dyestuffs. It is particularly suitable for dyeing cotton and regenerated cellulose with direct cotton dyestuffs.

10 The material used must be substantive to the dyestuff being used since the use of urea as a transfer medium in accordance with this invention does not extend the range of dyestuffs available for dyeing any particular type of textile material.

15 The process of the present invention is suitable for dyeing those organic textiles which are not deleteriously affected by baking at a temperature of 130 to 160° C. for example textile materials of cotton, wool, regenerated cellulose, artificial protein fibres, cellulose esters, for example secondary acetate and triacetate fibres, synthetic polyamides, synthetic polyesters, polyacrylonitrile and the like and materials made from mixtures of two or more of these fibres. It is not suitable for dyeing glass and other mineral fibres. If the process is used for dyeing

20 textiles from thermoplastic fibres having a comparatively low melting point for example certain vinyl resin fibres the baking should be carried out at the lower temperature and for the shortest time permissible.

I have found that, apart from the one class of easily 30 levelling acid dyes on nylon which requires strongly acid dyeing conditions, the process of this invention can be used with any dyestuff for which water is known to be a suitable transfer medium. Thus if it is known that a

35 dyestuff can be satisfactorily applied to a particular textile material from an aqueous dyebath, other than a strongly acid dyebath as in the case of the easily levelling acid dyestuffs, it can be assumed that it can also be applied to the same material using urea as a transfer medium in accordance with this invention. The following test may 40 however be used to determine whether any particular dyestuff is soluble in urea:

The method consists in blowing the dyestuff powder on to a dry filter paper which has previously been impregnated with a 50 percent aqueous solution of urea and 45 dried. The test paper is then placed for about 3 minutes in an oven which is maintained at a temperature slightly above 132° C. Coloured haloes are formed if the dyestuff is soluble in molten urea. Such a test does not define the degree of solubility but the actual degree of 50 solubility is immaterial; if the conditions specified in the test are satisfied, i.e. a coloured halo is formed, the dyestuff can be used in the process of this invention. When used in the specification and claims of this application, the term "dye which is soluble in molten urea" means a dye 55 which complies with the test set out above.

As in the case of dyeing from aqueous baths, two or more substantive dyestuffs may be applied simultaneously.

The following lists give examples of suitable dyes for 60 dyeing various textile materials (references are to the Color Index, second edition):

**FOR COTTON AND REGENERATED CELLULOSE**

Chlorantine Brown BRLL (Clayton Dyestuffs Ltd.) (C.I. Direct Brown 95)

65 Solophenyl Blue Green BL (Geigy) (C.I. Direct Green 27)

Durazol Red 2B (I.C.I.) (C.I. Direct Red 81)

Durazol Red 6B (I.C.I.) (C.I. Direct Red 79)

Durazol Orange 2G (I.C.I.) (C.I. Direct Orange 34)  
Diphenyl Chlorine Yellow FF (Geigy) (C.I. Direct Yellow 28),  
And related dyestuffs.

#### FOR CELLULOSE ACETATE

All dispersed dyes may be used. Examples are:

Serisol Brilliant Blue BG (C.I. Disperse Blue 3)<sup>1</sup>  
Duranol Red 2B (C.I. Disperse Red 15)<sup>1</sup>  
Dispersol Fast Yellow G (C.I. Disperse Yellow 3)<sup>1</sup>  
Dispersol Fast Orange G (J.S.D.C., 71, p. 505) (C.I. Disperse Orange 3)  
Dispersol Fast Crimson B (I.C.I.) (C.I. Disperse Red 13)  
Duranol Blue BN (I.C.I.) (C.I. Disperse Blue 3)  
Serisol Fast Scarlet GD (Yorkshire Dyeware & Chemical Co.) (C.I. Disperse Red 19)

Solubilised vat dyestuffs can also be used. Typical examples are:

Soledon Jade Green XS (I.C.I.) (C.I. solubilized vat green 1)  
Soledon Golden Yellow RKS (I.C.I.) (C.I. solubilized vat orange 1)

Sulphonated hydroxy-ethyl derivatives of certain dyes may also be used, for example the Solacet range of dyes by I.C.I.

#### FOR CELLULOSE TRIACETATE

The dispersed dyes and solubilised vat dyes, and those specifically given above under cellulose acetate, may also be used for the triacetate.

#### FOR POLYACRYLONITRILE FIBRES

Basic dyestuffs are applicable. Examples are:

Sevron Blue 2G (Brown & Forth) (C.I. Basic Blue 22)  
Sevron Yellow L (Brown & Forth) (C.I. Basic Yellow 13)

Dispersol Fast Crimson B (C.I. Disperse Red 13) is an example of a suitable dispersed dye. If the acrylic fibre contains a dyeable additive such as polyvinyl pyridine then the whole range of acid dyes may be used.

#### FOR NYLON

Dispersed dyes may be used. Examples are:

Serisol Fast Scarlet GD (Yorkshire Dyeware Chemical Co.) (C.I. Disperse Red 19)  
Serisol Brilliant Blue BG (Yorkshire Dyeware & Chemical Co.) (C.I. Disperse Blue 3)  
Dispersol Fast Crimson B (I.C.I.) (C.I. Disperse Red 13)

Sulphonated hydroxy-ethyl derivatives of dispersed dyes may be used. Examples are:

Solacet Fast Crimson B (I.C.I.) (C.I. Acid Red 159)  
Solacet Scarlet B (I.C.I.) (C.I. Acid Red 53)  
Solacet Fast Blue 2B (I.C.I.) (C.I. Acid Blue 14)

Metal complex dyes may be used. Examples are:

Vilon Yellow G (Allied Colloids Ltd.) (C.I. Acid Yellow 118)  
Vilon Fast Brown R (Allied Colloids Ltd.) (C.I. Acid Brown 50)

Solubilised vat dyestuffs may be used. Examples are:

Soledon Jade Green XS (I.C.I.) (C.I. solubilized vat green 1)  
Soledon Golden Yellow RKS (I.C.I.) (C.I. solubilized vat orange 1)

Aggregated dyestuffs may also be used. Examples are:

Coomassie Red PGS (I.C.I.) (C.I. Acid red 85)  
Carbolan Yellow RS (I.C.I.) (C.I. Acid yellow 71)  
Coomassie Fast Yellow GS (I.C.I.) (C.I. acid yellow 85)  
Carbolan Crimson BS (I.C.I.) (C.I. acid red 138)

#### FOR POLYESTERS (TERYLENE; DACRON)

Dispersed dyestuffs, particularly rapidly diffusing dyestuffs, may be used. Examples are:

Dispersol Fast Yellow G (I.C.I.) (C.I. Disperse Yellow 3)  
Dispersol Fast Orange G (I.C.I.) (C.I. Disperse Orange 3)  
Duranol Red GN (I.C.I.) (C.I. Disperse Red 9)  
Duranol Red 2B (I.C.I.) (C.I. Disperse Red 15)  
Duranol Violet 2R (I.C.I.) (C.I. Disperse Violet 1)

The textile materials may be dyed according to the process of the invention in any convenient form, for example, the process may be applied to woven or knitted fabrics or to threads, yarns or fibres.

Tests may be necessary to determine the optimum take-up of urea and the optimum length of time of baking for a particular dyestuff and for a particular textile material. The upper limit of the temperature of baking (160° C.) is determined by the tendency for urea to decompose at elevated temperatures.

Any suitable apparatus can be used to carry out the process, for example, the textile material may be impregnated with urea and a dyestuff from an aqueous solution on a pad mangle and the impregnated material may be dried and baked in an oven. The apparatus normally used for carrying out a crease-resist treatment with a urea-formaldehyde resin on textile materials can be used without substantial alteration.

The process of this invention using urea as transfer medium, compared with the customary technique using aqueous dyebaths, has several advantages. For example dye transfer with urea is considerably quicker, the urea process can be carried out in a continuous manner and is more economical, and also the urea process often gives levelness of dyeing where aqueous baths would not, for example in the dyeing of so-called "stripey fibres" where any differences in dyeing affinity are levelled out by using the urea process. The urea dyeing process does not substantially affect the strength of the fibres.

The invention is illustrated by the following examples.

#### Example 1

A sample of woven fabric containing 67 percent of viscose rayon staple fibres and 33 percent of regenerated protein staple fibres was padded at 110 percent expression through a solution at room temperature prepared as follows:

55 0.4 gram of Durazol Yellow GS (I.C.I.) (C.I. Direct Yellow 28)  
0.4 gram of Durazol Blue 2GNS (C.I. Direct Blue 76) (Journal of the Society of Dyers and Colourists, 1952, page 534), and  
40 grams of urea

were made up to 100 cubic centimetres with water. The sample was then dried at 80° C. in a circulating air oven and then baked for 10 minutes at 140° C. The dyed sample was washed for ten minutes in cold water and dried at 80° C.

A comparable dyeing carried out in accordance with normal practice was carried out on a second sample of the same material. The dyebath was an aqueous solution containing

0.4 percent of Durazol Yellow GS (I.C.I.)  
0.4 percent of Durazol Blue 2GNS (Journal of the Society of Dyers and Colourists, 1952, page 534)  
75 10 percent of Glauber's salt

<sup>1</sup> See Journal of Society of Dyers and Colourists, vol. 71, page 455.

All the percentages were based on the weight of the textile material, and the dyebath had a liquor to fabric ratio of 40:1. The dyeing was carried out for one hour at 90° C. The sample was then washed in cold water and dried at 80° C.

On comparing the two methods it was found that the fabric dyed by the process of the present invention was quite even, whereas the fabric dyed from an aqueous dyebath showed a degree of differential dyeing and was consequently unevenly coloured.

On subjecting the dyed fabrics to the washing test as described in the Second Report of the Fastness Tests Committee of the Society of Dyers and Colourists (Journal of the Society of Dyers and Colourists 1948, volume 64, pages 136-7, Test No. 1) it was found that the fabric dyed by the process of the present invention was of comparable fastness to the fabric dyed from an aqueous bath.

#### Example 2

A fabric woven from 100 percent viscose rayon staple yarn was padded at 110 percent expression through a solution at room temperature prepared as follows:

1 gram of Durazol Yellow 3RS (I.C.I.), and  
40 grams of urea

were made up to 100 cubic centimetres with water. The fabric was dried in a circulating air oven at 80° C. and then divided into two parts. One part was baked for 10 minutes at 150° C. and the other part was unbaked. On subjecting both the baked and unbaked fabrics to the washing test described in Example 1 it was found that the baked fabric substantially retained its shade and showed only slight bleeding on to an unstained cotton fabric present during the test; in contrast, the unbaked sample showed a severe loss in depth of shade.

#### Example 3

A fabric woven from 100 percent viscose rayon staple yarn was padded at 110 percent expression through a solution at room temperature prepared as follows:

1 gram of Durazol Rubine BS (I.C.I.) (C.I. Direct Red 82), and  
40 grams of urea

were made up to 100 cubic centimetres with water. After drying in a circulating air oven at 80° C., the fabric was divided into two parts, which were treated as described in Example 2. Similar results were obtained, the unbaked sample showing severe loss of colour; the baked sample showed substantially better retention of the dyestuff.

#### Example 4

A fabric 20 yards long and 36 inches wide woven from yarns of regenerated cellulose staple fibre was padded at 100 percent expression through an aqueous solution at room temperature containing

50 percent urea  
1.25 percent Chlorantine Brown BRLL 200 percent (Clayton Aniline Co.) (C.I. Direct Brown 95)  
1 percent Calsolene Oil

The fabric was dried for three minutes at 80° C. by a single passage through a circulating air drying chamber. The fabric was then baked by passing it again through the same chamber at 140° C. for three minutes. The cooled, baked fabric was washed for 15 minutes in water at 30° C. and finally dried at 80° C.

A smaller length was dyed to a similar shade on a winch using a dyebath containing

1.25 percent Chlorantine Brown BRLL 200 percent (on weight of fabric)  
20 percent Glauber's salt (on weight of fabric)

at a bath ratio of 40:1. The time of dyeing was 2½ hours and the temperature of the dyebath 90° C.

On subjecting both fabrics to the washing test as described in Example 1, it was found that the two fabrics were of comparable washing fastness.

Tests also showed that the two fabrics were of comparable light fastness.

#### Example 5

10 A circular knitted fabric containing 67 percent of wool and 33 percent of regenerated protein staple fibres was padded at 110 percent expression through a solution at room temperature prepared as follows:

15 0.4 gram of Carbolan Yellow 3G 113 percent (C.I. Acid Yellow 72) (Theory and Practice of Wool Dyeing, C. L. Byrd, 1947, page 55)

1.2 grams of Carbolan Blue RS (C.I. Acid Blue 159) (Journal of the Society of Dyers and Colourists, 1947, page 283)

0.4 gram of Carbolan Crimson BS (C.I. Acid Red 138) (Theory and Practice of Wool Dyeing, C. L. Bird, 1947, page 55)

20 2 grams of Calsolene Oil, and  
25 40 grams of urea

were made up to 100 cubic centimetres with water. The material was then dried in a circulating air oven at 80° C. and baked for 10 minutes at 140° C. Another sample of the same fabric was padded similarly through a solution made up as above but with the urea omitted, and dried and baked as described.

On subjecting to the washing test described in Example 1, it was found that the sample padded without urea showed severe loss of colour, whereas the sample padded with urea showed satisfactory retention and exhibited no bleeding on to undyed wool and cotton fabrics present during the test.

#### Example 6

A cutting of warp knitted nylon fabric was padded through a solution at room temperature prepared as follows:

45 1 gram of Vialon Yellow G (C.I. Acid Yellow 118) (Badische Anilin & Soda Fabrik)  
2 grams of Calsolene Oil, and  
40 grams of urea

were made up to 100 cubic centimetres with water. The fabric was dried in a circulating air oven at 80° C. and baked for 10 minutes at 150° C. A further portion of fabric was padded through a solution made up as above, but with the urea omitted, and similarly dried and baked. On washing in cold water it was found that the fabric padded without the inclusion of urea showed marked loss of dyestuff and gave only a pale shade. The presence of urea resulted in a shade of substantially greater tinctorial value.

#### Example 7

A padding solution was prepared as follows:

50 parts urea,  
3 parts Duranol Violet 2R 300 (I.C.I.) (C.I. Acid Violet 1),

65 1 part sodium carboxymethyl cellulose,  
1 part Dispersol VL (a non-ionic dispersing agent sold by Imperial Chemical Industries Ltd.)

made up to 100 part with water.

A fabric woven from yarns of polyester fibres sold under the registered trademark "Terylene" was padded through this solution at 35 percent expression, dried for three minutes at 80° C., baked for three minutes at 145° C., washed in water at room temperature and dried at 80° C.

A similar piece of fabric was pot dyed for 1½ hours at the boil using an aqueous dyebath containing:  
1 percent Duranol Violet 2R 300 (I.C.I.), and  
5 percent Dispersol VL (I.C.I.),

at a bath ratio of 40:1.

On subjecting both fabrics to the washing test described in Example 1 it was found that both fabrics were of good wash fastness (4 to 5), the urea dyed fabric showing slightly greater fastness.

#### Examples 8 to 10

Further samples of "Terylene" fabrics as used in Example 7 were dyed in the same way as described in Example 7 except that the padding solution contained, instead of three parts of Duranol Violet 2R 300,

Example 8: 3 parts of Dispersol F Yellow G 300 (I.C.I.) (C.I. Disperse Yellow 3)

Example 9: 3 parts of Dispersol F Orange G 300 (I.C.I.) (C.I. Disperse Orange 3)

Example 10: 3 parts of Duranol Blue 2GN 300 (I.C.I.) (C.I. Disperse Blue 24).

Other pieces of "Terylene" fabric were dyed to the same shade using the conventional pot dyeing method described in Example 7. By subjecting the fabrics to the washing test referred to in Example 1, all the fabrics were found to be of good wash fastness (4 to 5) with the urea dyed fabrics showing slightly greater fastness. In addition microscopic examination of yarn from the dyed fabrics showed that the depth of penetration of dyestuff into the filaments was greater using the method according to the invention.

#### Example 11

A cutting of plain woven continuous filament cellulose acetate fabric was padded at 70 percent expression through an aqueous solution at room temperature containing

1.4 parts Dispersol Yellow G 300 (I.C.I.) (C.I. Disperse Yellow 3)

45 parts urea, and

2 parts Calsolene Oil HS,

made up to 100 parts with water.

The cutting was then dried at 80° C. and baked for four minutes at 145° C. It was afterwards rinsed in cold water. A further cutting was dyed to a similar shade using an aqueous dyebath containing 1 percent Dispersol Yellow G 300. The bath ratio was 40:1 and the time and temperature of dyeing ¾ hour at 80° C. On subjecting to the washing test as described in Example 1, it was found that both fabrics exhibited a similar wash fastness.

#### Example 12

A cutting of the fabric similar to that used in Example 11 was padded and baked as described in that example using Duranol Blue Green B (I.C.I.) (C.I. Disperse Blue 7) in place of Dispersol Yellow G. A further cutting was dyed from an aqueous bath again as described in Example 11 but using Duranol Blue Green B in place of Dispersol Yellow G. On subjecting the dyed fabrics to the washing test as described in Example 1, both fabrics showed wash fastness of a similar order.

#### Example 13

A cutting bleached plain woven 100 percent cotton fabric was padded through an aqueous solution at room temperature containing

1 part Chlorantine Brown BRLL 200 percent (Clayton Aniline Co) (C.I. Direct Brown 95), and

45 parts urea,

made up to 100 parts with water.

The cutting was dried at 80° C., baked for four minutes

at 145° C., and rinsed in cold water. A second cutting was dyed from an aqueous bath containing

1 percent Chlorantine Brown BRLL (on weight of fabric),  
10 percent Glauber's salt (on weight of fabric).

The bath ratio was 40:1 and the time and temperature of dyeing ¾ hour at 90° C. On subjecting the dyed fabrics to the washing test as described in Example 1, the wash fastness of both samples was found to be similar.

#### Example 14

The dyeings and tests described in Example 13 were repeated using instead of Chlorantine Brown BRLL, Chlorantine Green 5GLL (C.I. Direct Green 28). Again the dyed fabrics were of comparable wash fastness.

#### Example 15

A cutting of fabric woven from 100 percent viscose rayon staple was padded, at room temperature, through a solution containing

1 gram Solochrome Azurine B (C.I. Mordant Blue 1), (I.C.I.),

2 cubic centimetre basic chromium acetate (32° Tw), and 50 grams urea,

made up to 100 cubic centimetres with water.

The cutting was dried at 80° C., baked for four minutes at 145° C., and finally washed in cold water. As dried, the fabric was a beige colour but turned blue during the baking stage. On submitting the fabric to the washing test, as described in Example 1, it was found that a satisfactory wash fastness had been obtained. Filaments taken from the fabric were examined in cross-section under the microscope, and the dyestuff was seen to be deposited throughout the filaments.

#### Example 16

A cutting of knitted fabric made from cellulose acetate yarn was padded through a solution containing

1 gram Soledon Jade Green 2GS, (I.C.I.) (C.I.) solubilized vat green 2), and

50 grams urea,

made up to 100 cubic centimeters with water.

It was then dried at 80° C., baked for four minutes at 145° C., and washed in cold water. During the baking stage the colour of the fabric changed from violet-brown (the colour of the leuco ester of the dyestuff) to green, the colour of the parent dyestuff. No significant change of shade was evident after treatment for ½ hour at 80° C. in 0.2 percent soap solution.

It has been found that certain leuco-esters of vat dyestuffs do not show this reversion to the shade of the parent dyestuff on baking. In these cases orthodox methods of regeneration may be carried out after baking, for example atmospheric oxidation, or oxidation by means of oxidising agents.

#### Example 17

A knitted fabric made from cellulose triacetate yarn was padded through a solution containing

1 gram of Serisol Brilliant Blue BG (C.I. Disperse Blue 3), and

50 grams of urea,

made up to 100 cubic centimetres with water.

The fabric was dried at 80° C., baked for four minutes at 145° C., washed in water and dried. The fabric was dyed blue.

#### Example 18

A knitted fabric made from yarn consisting of a polymer of 95 percent of acrylonitrile and 6 percent of methyl acrylate was padded through a solution containing

1 gram of Sevron Blue 2G (C.I. basic blue 22), and

50 grams of urea,

made up to 100 cubic centimetres with water.

The fabric was dried at 80° C., baked for four minutes at 145° C., washed in water and dried. The fabric was dyed blue.

In the baking step in the process of the present invention the urea melts and acts as a dye transfer medium. The process of the present invention provides a simple and convenient alternative to the established practice of dyeing from aqueous dyebaths. The process is simple, quick, easy to control and eliminates many of the difficulties encountered in dyeing with aqueous dyebaths.

The process is particularly suitable for dyeing blends of two or more different fibres especially where one of the fibres shows a preferential absorption for the dyestuff from an aqueous dyebath, for example blends of viscose rayon fibres and regenerated protein fibres can be dyed in an even shade with a direct cotton dyestuff by the process of the present invention whereas the blends would be differentially dyed from an aqueous dyebath.

The process is also particularly suitable for dyeing textile materials of synthetic polyesters, for example of polyethylene terephthalate.

What I claim is:

1. A process for dyeing organic textile materials which endure baking at 130° C.-160° C. which comprises impregnating the textile material with a solution of urea and with an aqueous solution or dispersion of at least one dyestuff which is soluble in molten urea and is substantive to the textile material, drying the textile material at a temperature below the melting point of the urea, heating the dried material in the absence of steam at a temperature sufficient to melt the urea and not higher than

160° C. whereby the urea is melted and serves as a solvent for the dyestuff, from which resultant solution transfer of the dyestuff to the material takes place, washing the dyed material to remove the urea and again drying the material.

5 2. A process as claimed in claim 1 wherein the solution of urea used is an aqueous solution.

3. A process as claimed in claim 1 wherein the textile material is impregnated with a single solution of urea in which the dyestuff is dissolved or dispersed.

10 4. A process as claimed in claim 1 wherein the textile materials dyed comprise regenerated cellulose.

5. A process as claimed in claim 1 wherein the textile materials dyed comprise wool.

15 6. A process as claimed in claim 1 wherein the textile materials dyed comprise nylon.

7. A process as claimed in claim 1 wherein the textile materials dyed comprise cellulose acetate.

20 8. A process as claimed in claim 1 wherein the textile materials dyed comprise acrylic fibre.

#### References Cited in the file of this patent

##### UNITED STATES PATENTS

25 1,963,975 Ellis \_\_\_\_\_ June 26, 1934  
2,080,254 Dreyfus \_\_\_\_\_ May 11, 1937

##### FOREIGN PATENTS

996,335 France \_\_\_\_\_ Dec. 18, 1951  
30 505,597 Canada \_\_\_\_\_ Sept. 7, 1954  
230,891 Switzerland \_\_\_\_\_ May 16, 1944